



US009574256B2

(12) **United States Patent**  
**Imataka et al.**

(10) **Patent No.:** **US 9,574,256 B2**  
(45) **Date of Patent:** **Feb. 21, 2017**

(54) **STEEL FOR COLD FORGING/NITRIDING, STEEL MATERIAL FOR COLD FORGING/NITRIDING, AND COLD-FORGED/NITRIDED COMPONENT**

(71) Applicant: **NIPPON STEEL & SUMITOMO METAL CORPORATION**, Tokyo (JP)

(72) Inventors: **Hideki Imataka**, Tokyo (JP); **Masayuki Horimoto**, Tokyo (JP); **Yuya Gyotoku**, Tokyo (JP); **Kosuke Tanaka**, Tokyo (JP)

(73) Assignee: **NIPPON STEEL & SUMITOMO METAL CORPORATION**, Tokyo (JP)

(\*) Notice: Subject to any disclaimer, the term of this patent is extended or adjusted under 35 U.S.C. 154(b) by 154 days.

(21) Appl. No.: **14/389,776**

(22) PCT Filed: **Feb. 28, 2013**

(86) PCT No.: **PCT/JP2013/055296**

§ 371 (c)(1),  
(2) Date: **Oct. 1, 2014**

(87) PCT Pub. No.: **WO2013/150844**

PCT Pub. Date: **Oct. 10, 2013**

(65) **Prior Publication Data**

US 2015/0059933 A1 Mar. 5, 2015

(30) **Foreign Application Priority Data**

Apr. 2, 2012 (JP) ..... 2012-083609

(51) **Int. Cl.**  
**C22C 38/02** (2006.01)  
**C22C 38/60** (2006.01)

(Continued)

(52) **U.S. Cl.**  
CPC ..... **C22C 38/60** (2013.01); **C21D 9/0075** (2013.01); **C22C 38/001** (2013.01);  
(Continued)

(58) **Field of Classification Search**  
CPC ..... **C22C 38/02**  
(Continued)

(56) **References Cited**

U.S. PATENT DOCUMENTS

2012/0048427 A1 3/2012 Kubota

FOREIGN PATENT DOCUMENTS

CN 102089452 6/2011  
ES EP 1876255 A1 \* 1/2008 ..... C22C 38/02  
(Continued)

Primary Examiner — Brian Walck

(74) Attorney, Agent, or Firm — Clark & Brody

(57) **ABSTRACT**

A steel comprises, by mass percent, C: 0.10 to 0.15%, Si: not less than 0.02% and less than 0.10%, Mn: more than 0.90% and not more than 2.50%, P≤0.030%, S≤0.050%, Cr: 0.80 to 2.0%, V: 0.05 to 0.50%, Al: 0.01 to 0.07%, N≤0.0080%, O≤0.0030%, and one or more selected from Mo, Cu, Ni, Ti, Nb, Zr, Pb, Ca, Bi, Te, Se and Sb, the balance being Fe and impurities. The composition satisfies  $[35 \leq \text{Mn}/\text{S} \leq 200]$ ,  $[20 \leq (669.3 \times \log_e \text{C} - 1959.6 \times \log_e \text{N} - 6983.3) \times (0.067 \times \text{Mo} + 0.147 \times \text{V}) \leq 80]$ ,  $[140 \times \text{Cr} + 125 \times \text{Al} + 235 \times \text{V} \geq 160]$  and  $[150 \leq 511 \times \text{C} + 33 \times \text{Mn} + 56 \times \text{Cu} + 15 \times \text{Ni} + 36 \times \text{Cr} + 5 \times \text{Mo} + 134 \times \text{V} \leq 200]$ .

**6 Claims, 12 Drawing Sheets**



|                      |                                                                                                                                                                                                                                                                                                                            |    |                 |                                                                                                                                                                                                                                                                                                                                      |
|----------------------|----------------------------------------------------------------------------------------------------------------------------------------------------------------------------------------------------------------------------------------------------------------------------------------------------------------------------|----|-----------------|--------------------------------------------------------------------------------------------------------------------------------------------------------------------------------------------------------------------------------------------------------------------------------------------------------------------------------------|
| (51) <b>Int. Cl.</b> |                                                                                                                                                                                                                                                                                                                            |    |                 |                                                                                                                                                                                                                                                                                                                                      |
| <i>C23C 8/02</i>     | (2006.01)                                                                                                                                                                                                                                                                                                                  |    |                 | (2013.01); <i>C22C 38/26</i> (2013.01); <i>C22C 38/28</i> (2013.01); <i>C22C 38/38</i> (2013.01); <i>C22C 38/42</i> (2013.01); <i>C22C 38/46</i> (2013.01); <i>C22C 38/50</i> (2013.01); <i>C22C 38/58</i> (2013.01); <i>C23C 8/02</i> (2013.01); <i>C23C 8/26</i> (2013.01); <i>C23C 8/50</i> (2013.01); <i>C21D 7/02</i> (2013.01) |
| <i>C23C 8/26</i>     | (2006.01)                                                                                                                                                                                                                                                                                                                  |    |                 |                                                                                                                                                                                                                                                                                                                                      |
| <i>C21D 9/00</i>     | (2006.01)                                                                                                                                                                                                                                                                                                                  |    |                 |                                                                                                                                                                                                                                                                                                                                      |
| <i>C22C 38/00</i>    | (2006.01)                                                                                                                                                                                                                                                                                                                  |    |                 |                                                                                                                                                                                                                                                                                                                                      |
| <i>C22C 38/06</i>    | (2006.01)                                                                                                                                                                                                                                                                                                                  |    |                 |                                                                                                                                                                                                                                                                                                                                      |
| <i>C22C 38/20</i>    | (2006.01)                                                                                                                                                                                                                                                                                                                  |    |                 |                                                                                                                                                                                                                                                                                                                                      |
| <i>C22C 38/24</i>    | (2006.01)                                                                                                                                                                                                                                                                                                                  |    |                 |                                                                                                                                                                                                                                                                                                                                      |
| <i>C22C 38/38</i>    | (2006.01)                                                                                                                                                                                                                                                                                                                  |    |                 |                                                                                                                                                                                                                                                                                                                                      |
| <i>C22C 38/46</i>    | (2006.01)                                                                                                                                                                                                                                                                                                                  |    |                 |                                                                                                                                                                                                                                                                                                                                      |
| <i>C22C 38/58</i>    | (2006.01)                                                                                                                                                                                                                                                                                                                  |    |                 |                                                                                                                                                                                                                                                                                                                                      |
| <i>C22C 38/22</i>    | (2006.01)                                                                                                                                                                                                                                                                                                                  |    |                 |                                                                                                                                                                                                                                                                                                                                      |
| <i>C22C 38/26</i>    | (2006.01)                                                                                                                                                                                                                                                                                                                  |    |                 |                                                                                                                                                                                                                                                                                                                                      |
| <i>C22C 38/28</i>    | (2006.01)                                                                                                                                                                                                                                                                                                                  |    |                 |                                                                                                                                                                                                                                                                                                                                      |
| <i>C22C 38/42</i>    | (2006.01)                                                                                                                                                                                                                                                                                                                  | JP | 05-171347       | 7/1993                                                                                                                                                                                                                                                                                                                               |
| <i>C22C 38/50</i>    | (2006.01)                                                                                                                                                                                                                                                                                                                  | JP | 07-102343       | 4/1995                                                                                                                                                                                                                                                                                                                               |
| <i>C23C 8/50</i>     | (2006.01)                                                                                                                                                                                                                                                                                                                  | JP | 09-71841        | 3/1997                                                                                                                                                                                                                                                                                                                               |
| <i>C21D 7/02</i>     | (2006.01)                                                                                                                                                                                                                                                                                                                  | JP | 10-306343       | 11/1998                                                                                                                                                                                                                                                                                                                              |
| (52) <b>U.S. Cl.</b> |                                                                                                                                                                                                                                                                                                                            | JP | 2004-238702     | 8/2004                                                                                                                                                                                                                                                                                                                               |
| CPC .....            | <i>C22C 38/002</i> (2013.01); <i>C22C 38/02</i> (2013.01); <i>C22C 38/06</i> (2013.01); <i>C22C 38/20</i> (2013.01); <i>C22C 38/22</i> (2013.01); <i>C22C 38/24</i> (2013.01); <i>C22C 38/26</i> (2013.01); <i>C23C 8/02</i> (2013.01); <i>C23C 8/26</i> (2013.01); <i>C23C 8/50</i> (2013.01); <i>C21D 7/02</i> (2013.01) | JP | 2004-300473     | 10/2004                                                                                                                                                                                                                                                                                                                              |
|                      |                                                                                                                                                                                                                                                                                                                            | JP | EP 1577406 A1 * | 9/2005 .....                                                                                                                                                                                                                                                                                                                         |
|                      |                                                                                                                                                                                                                                                                                                                            | JP | 2006-063378     | 3/2006                                                                                                                                                                                                                                                                                                                               |

(58) **Field of Classification Search**

USPC ..... 148/318; 420/104-112  
See application file for complete search history.

(56) **References Cited**

## FOREIGN PATENT DOCUMENTS

|    |                 |              |
|----|-----------------|--------------|
| JP | 05-171347       | 7/1993       |
| JP | 07-102343       | 4/1995       |
| JP | 09-71841        | 3/1997       |
| JP | 10-306343       | 11/1998      |
| JP | 2004-238702     | 8/2004       |
| JP | 2004-300473     | 10/2004      |
| JP | EP 1577406 A1 * | 9/2005 ..... |
| JP | 2006-063378     | 3/2006       |

\* cited by examiner

FIG 1



FIG 2



FIG 3



FIG 4



FIG 5



FIG 6



FIG 7



FIG 8



FIG 9



FIG 10



FIG 11



FIG 12

→ : Measuring direction of wear depth



FIG 13

Indentation test jig



FIG 14



FIG 15



FIG 16



FIG 17



FIG 18



FIG 19



**STEEL FOR COLD FORGING/NITRIDING,  
STEEL MATERIAL FOR COLD  
FORGING/NITRIDING, AND  
COLD-FORGED/NITRIDED COMPONENT**

**TECHNICAL FIELD**

The present invention relates to a steel for cold forging/nitriding, a steel material for cold forging/nitriding, and a cold-forged/nitrided component. More specifically, the present invention relates to a steel for cold forging/nitriding and a steel material for cold forging/nitriding, which are excellent in cold forge ability and machinability (particularly, chip disposability) after cold forging, and also can provide a component subjected to a cold forging and nitriding treatment with high core hardness and high surface hardness and a large effective case depth, and are used suitably as a starting material for a cold-forged/nitrided component, and a cold-forged/nitrided component using the same.

The “nitriding” in the present invention is a treatment including the “nitrocarburizing” treatment in which “N and C are caused to invade and diffuse”, not merely the “nitriding” treatment in which “N is caused to invade and diffuse”. Therefore, in the explanation below, a treatment including the “nitrocarburizing” is referred simply to as the “nitriding”.

In addition, the “cold forging/nitriding” means a treatment in which the “cold forging” has been carried out, and then the “nitriding” treatment is further carried out.

**BACKGROUND ART**

A component for machine structural use that is used for an automobile transmission and the like, such as a gear and a pulley for a belt-type continuously variable transmission (CVT), is usually subjected to surface hardening treatments from the viewpoint of improving bending fatigue strength, pitting strength, and wear resistance. There are typical surface hardening treatments such as “carburizing and quenching”, “induction quenching”, and “nitriding”.

Among the treatments mentioned above, the “carburizing and quenching” is a treatment in which a low carbon steel is generally used; and in the said treatment, C is caused to invade and diffuse in an austenitic region of a high temperature not less than the  $Ac_3$  point, and thereafter quenching is carried out. The “carburizing and quenching” has an advantage of attaining a high surface hardness and a large effective case depth, but this treatment is accompanied by phase transformation; and thus in the said treatment, there is a problem that the heat treatment distortion becomes large. Therefore, in the case where the high component accuracy is required, it is necessary to carry out a finish working, which is grinding, honing and so on, after the “carburizing and quenching”. In addition, the “carburizing and quenching” has a problem that a so-called “abnormal carburized layer”, which is an intergranularly oxidized layer, non-martensitic layer and so on, produced on the outer layer becomes a start point of failure such as bending fatigue failure, and the fatigue strength is deteriorated.

The “induction quenching” is a treatment in which a steel is rapidly heated to an austenitic region of a high temperature not less than the  $Ac_3$  point and thereafter quenched. The “induction quenching” has an advantage that the effective case depth can be controlled with relative ease, but this treatment is not a surface hardening treatment in which C is caused to invade and diffuse like the carburizing treatment. Therefore, in the case of the “induction quenching”, in order

to attain necessary surface hardness, effective case depth and core hardness, a medium carbon steel, which has a higher C content as compared with a steel for carburizing treatment, is generally used. However, as for a starting material, the medium carbon steel has a higher hardness than the low carbon steel; and thus there is a problem that steels for the said “induction quenching” are inferior in machinability. In addition, with regard to the “induction quenching”, a high frequency heating coil must be prepared for each component.

In contrast, the “nitriding” is a treatment in which N is caused to invade and diffuse at a temperature of about 400 to 550° C. not more than the  $Ac_1$  point, and thereby a high surface hardness and a proper effective case depth are attained. In the case of the “nitriding”, as compared with the “carburizing and quenching” and the “induction quenching”, the treatment temperature is low; and therefore the said “nitriding” has an advantage that the heat treatment distortion is small.

In addition, in the “nitriding”, the “nitrocarburizing” is a treatment in which N and C are caused to invade and diffuse at a temperature of about 500 to 650° C. not more than the  $Ac_1$  point, and thereby a high surface hardness is attained. This treatment is suitable for mass production because the treatment time is as short as several hours.

Furthermore, along with the trend toward the reduction in greenhouse gas with the recent restraint of global warming being a background, it has been demanded that a process in which a steel is held at a high temperature, such as “carburizing and quenching”, be reduced. Therefore, the “nitriding” is a treatment responding to the demand of the day.

Unfortunately, the conventional steel for nitriding has problems described in the following <1> to <3>.

<1> The “nitriding” is a surface hardening treatment in which quenching from an austenitic region of a high temperature is not performed, that is to say, it is a surface hardening treatment in which strengthening accompanied by the martensitic transformation cannot be performed. Therefore, in order to provide a nitrided component with the desired core hardness, it is necessary to contain a large amount of alloying elements, and thus it is necessary to perform forming by hot forging or the like because it is difficult to perform forming by cold forging.

<2> As for a typical steel for nitriding, the “Aluminum Chromium Molybdenum Steel (SACM645)” specified in JIS G 4053 (2008) is available. With regard to the steel of this type, unfortunately, although a high surface hardness can be attained because Cr, Al and the like produce nitrides near the surface, a high bending fatigue strength cannot be attained because of a shallow effective case depth.

<3> In the nitrocarburizing of the nitriding, a component is held in a temperature range of about 500 to 650° C. for several hours; and thus the core of the said component is liable to be softened by tempering. As a result, for a component to which a high contact pressure is applied, plastic deformation is easily produced in the core, and the contact surface is depressed and deformed.

Accordingly, in order to solve the problems mentioned above, for example, the Patent Literatures 1 and 2 disclose techniques concerning the “nitriding”.

The Patent Literature 1 discloses a “steel for nitrocarburizing excellent in cold forgeability” having an objective of providing a steel for nitrocarburizing that has a hardness after rolling of 200 or less in Vickers hardness, and is excellent in nitrocarburizing property and cold forgeability. The aforementioned “steel for nitrocarburizing” consists, by mass percent, of C: 0.05 to 0.25%, Si: 0.50% or less, Mn:

0.55% or less, Cr: 0.50 to 2.00%; V: 0.02 to 0.35%, and Al: 0.005 to 0.050%, and further according to need Nb: 0.02 to 0.35%, with the balance being Fe and impurities.

The Patent Literature 2 discloses a “method for producing a nitrided component” by which a hard surface hardened layer, a large effective case depth, and the necessary core hardness can be obtained and in which the amount of machining such as cutting can be reduced. The aforementioned “method for producing a nitrided component” provides a technique in which a steel material having a chemical composition consisting, by mass percent, of C: 0.10 to 0.40%, Si: 0.10 to 0.70%, Mn: 0.20 to 1.50%, Cr: 0.50 to 2.50%, and V: 0.05 to 0.60%, and further according to need one or more of Al, Mo, Ti, Nb, Ta, B, S, Pb, Te, Se, Ca, Bi and Sb, with the balance being substantially Fe is subjected, before nitriding treatment, to heat treatment in which the precipitation of V is controlled, subsequently being subjected to a cold working, and is further subjected to a nitriding treatment.

#### LIST OF PRIOR ART DOCUMENT

##### Patent Literatures

Patent Literature 1: JP 5-171347 A

Patent Literature 2: JP 7-102343 A

#### SUMMARY OF THE INVENTION

##### Problems to be Solved by the Invention

The steel disclosed in the Patent Literature 1 is not necessarily excellent in all of cold forgeability, machinability after cold forging, deformation resistance, bending fatigue strength, and wear resistance. In addition, the effective case depth means a depth having a Vickers hardness (hereinafter, sometimes referred to as the “HV”) of 400 or more, so that it cannot be said that the steel has a sufficient effective case depth.

The steel disclosed in the Patent Literature 2 contains a large amount of alloying elements. Therefore, if cold forging is carried out at a high working ratio, sufficient cold forgeability cannot necessarily be attained, which sometimes brings a problem.

The present invention has been made in view of the above-described situations, and accordingly the objectives thereof are to provide a steel for cold forging/nitriding and a steel material for cold forging/nitriding, which are excellent in cold forgeability and machinability (particularly, chip disposability) after cold forging, and also can provide a component subjected to a cold forging and nitriding treatment with high core hardness and high surface hardness and a large effective case depth, and are used suitably as a starting material for a cold-forged/nitrided component.

In the concrete, the objectives of the present invention are to provide a steel for cold forging/nitriding and a steel material for cold forging/nitriding, which hardly generate cracks during cold forging and are excellent in chip disposability after cold forging, and further can attain the following hardness properties after cold forging and nitriding; the core hardness: 200 or more in HV, the surface hardness: 700 or more in HV, and the effective case depth: 0.20 mm or more; and thus can be used as a starting material for a cold-forged/nitrided component.

Another objective of the present invention is to provide a cold-forged/nitrided component using the said steel for cold forging/nitriding and steel material for cold forging/nitriding.

#### Means for Solving the Problems

As described before, the “nitriding” is a surface hardening treatment in which quenching from an austenitic region is not performed; that is to say, it is a surface hardening treatment in which strengthening accompanied by the martensitic transformation cannot be performed. Therefore, in order to provide a nitrided component with the desired core hardness, it is necessary to contain a large amount of alloying elements. However, in this case, it is difficult to perform forming by cold forging.

Accordingly, in order to solve the above problem, the present inventors first studied a means for attaining the core hardness, surface hardness, and effective case depth, which are necessary to a component for machine structural use, with forming by cold forging and performing surface hardening treatment by nitriding.

As a result, the present inventors arrived at a technical idea that excellent cold forgeability can be attained by keeping the amount of alloying elements to a necessary minimum, and thus a high core hardness can be attained by a combined effect of a work hardening due to the cold forging and an age hardening at the nitriding temperature.

Consequently, based on the above-described technical idea, the present inventors further carried out experiments repeatedly, and obtained the following findings (a) to (e).

(a) If Cr and Al are contained in the steel, the surface hardness can be increased by nitriding.

(b) In order to attain a higher surface hardness by nitriding and to increase the amount of age hardening at the nitriding temperature, it is effective to contain V in the steel while the content of N in the steel is restricted. If Mo is contained in the above mentioned steel, a larger amount of age hardening can be attained.

(c) In order to attain excellent cold forgeability, it is effective to restrict the occurrence of coarse MnS. The occurrence of coarse MnS can be restricted by restricting the ratio of the Mn content to the S content (Mn/S) to a specific range.

(d) If the contents of C, Mn, Cu, Ni, Cr, Mo and V in the steel are restricted to a specific range, excellent machinability can be provided after cold forging.

(e) By the work hardening due to the cold forging and age hardening during the nitriding, a high core hardness necessary as a component for machine structural use can be attained.

The present invention has been accomplished on the basis of the above-described findings. The main points of the present invention are the steels for cold forging/nitriding described below, the steel material for cold forging/nitriding described below, and the cold-forged/nitrided component described below.

(1) A steel for cold forging/nitriding, having a chemical composition comprising, by mass percent, C: 0.10 to 0.15%, Si: not less than 0.02% and less than 0.10%, Mn: more than 0.90% and not more than 2.50%, Cr: 0.80 to 2.0%, V: 0.05 to 0.50%, and Al: 0.01 to 0.07%, with the balance being Fe and impurities, wherein

P, S, N and O among the impurities are P: 0.030% or less, S: 0.050% or less, N: 0.0080% or less, and O: 0.0030% or less,

the Fn1 expressed by the formula (1) described below is 35 to 200,

the Fn2 expressed by the formula (2) described below is 20 to 80,

the Fn3 expressed by the formula (3) described below is 160 or more, and

the Fn4 expressed by the formula (4) described below is 150 to 200:

$$Fn1=Mn/S$$

(1);

$$Fn2=(669.3 \times \log_e C - 1959.6 \times \log_e N - 6983.3) \times (0.067 \times Mo + 0.147 \times V)$$

(2);

$$Fn3=140 \times Cr + 125 \times Al + 235 \times V$$

(3); and

$$Fn4=511 \times C + 33 \times Mn + 56 \times Cu + 15 \times Ni + 36 \times Cr + 5 \times Mo + 134 \times V$$

(4);

where, each symbol C, Mn, S, Cr, Mo, V, N, Al, Cu and Ni in the above formulas (1) to (4) represents the content by mass percent of the element concerned.

(2) The steel for cold forging/nitriding according to the above item (1), which contains, by mass percent, Mo: 0.50% or less in lieu of a part of Fe.

(3) The steel for cold forging/nitriding according to the above item (1) or (2), which contains, by mass percent, one or more elements selected from Cu: 0.50% or less and Ni: 0.50% or less in lieu of a part of Fe.

(4) The steel for cold forging/nitriding according to any one of the above items (1) to (3), which contains, by mass percent, one or more elements selected from Ti: 0.20% or less, Nb: 0.10% or less, and Zr: 0.10% or less in lieu of a part of Fe.

(5) The steel for cold forging/nitriding according to any one of the above items (1) to (4), which contains, by mass percent, one or more elements selected from Pb: 0.50% or less, Ca: 0.010% or less, Bi: 0.30% or less, Te: 0.30% or less, Se: 0.30% or less, and Sb: 0.30% or less in lieu of a part of Fe.

(6) A steel material for cold forging/nitriding having a chemical composition according to any one of the above items (1) to (5), wherein the content of V in precipitates determined by the extraction residue analysis is 0.10% or less.

(7) A cold-forged/nitrided component having a chemical composition according to any one of the above items (1) to (5), wherein the core hardness thereof is 200 or more in Vickers hardness, the surface hardness thereof is 700 or more in Vickers hardness, and the effective case depth thereof is 0.20 mm or more.

The term "impurities" so referred to in the phrase "the balance being Fe and impurities" indicates those elements which come from the raw materials such as ore and scrap, and/or the production environment when the steel is produced on an industrial scale.

#### Advantageous Effects of the Invention

The steel for cold forging/nitriding and the steel material for cold forging/nitriding of the present invention are excellent in cold forgeability and machinability (particularly, chip disposability) after cold forging, and also can provide a component subjected to a cold forging and nitriding treatment with high core hardness and high surface hardness and a large effective case depth. Therefore, the steel for cold forging/nitriding and the steel material for cold forging/nitriding of the present invention are used suitably as a starting material for a cold-forged/nitrided component.

In addition, the cold-forged/nitrided component of the present invention is excellent in deformation resistance, bending fatigue strength, and wear resistance; and therefore it can be used suitably as a component for machine structural use that is used for an automobile transmission and the like, such as a gear and a pulley for a CVT.

#### BRIEF DESCRIPTION OF THE DRAWINGS

FIG. 1 is a view showing a shape of a notched test piece for measuring critical compression ratio at the time of cold forging used in the EXAMPLES. In this figure, the units of the dimensions are "mm".

FIG. 2 is a view showing a shape of a round bar test piece for measuring hardness and so on after nitriding used in the EXAMPLES. In this figure, the units of the dimensions are "mm".

FIG. 3 is a view showing a rough shape of a notched Ono type rotating bending fatigue test piece as cut off condition from a cold drawn material used in the EXAMPLES. In this figure, except for the symbols "3.2S", the units of the dimensions are "mm".

FIG. 4 is a view showing a shape of a block test piece A for investigating wear resistance used in the EXAMPLES. The units of the dimensions that units are not indicated in this figure are "mm".

FIG. 5 is a view showing a shape of a block test piece B for investigating deformation resistance used in the EXAMPLES. The units of the dimensions that units are not indicated in this figure are "mm".

FIG. 6 is a diagram showing the heat pattern of nitrocarburizing carried out on the test pieces shown in FIGS. 2 to 5 in the EXAMPLES.

FIG. 7 is a view showing a finished shape of a notched Ono type rotating bending fatigue test piece used in the EXAMPLES. In this figure, the units of the dimensions are "mm".

FIG. 8 is a view for explaining the length of a chip produced by turning using an NC lathe in the EXAMPLES.

FIG. 9 is a view for explaining a method for a block-on-ring wear test carried out in the EXAMPLES.

FIG. 10 is a view showing a shape of a ring test piece used for the block-on-ring wear test in the EXAMPLES. The units of the dimensions that units are not indicated in this figure are "mm".

FIG. 11 are diagrams showing the heat patterns of gas "carburizing and quenching" and tempering carried out on the ring test piece and the indentation test jig before finish grinding in the EXAMPLES.

FIG. 12 is a view for explaining a method for measuring a wear depth after the block-on-ring wear test carried out in the EXAMPLES.

FIG. 13 is a view for explaining a method for an indentation test carried out in the EXAMPLES.

FIG. 14 is a view showing a shape of an indentation test jig used for the indentation test in the EXAMPLES. The units of the dimensions that units are not indicated in this figure are "mm".

FIG. 15 is a graph summarizing the relationship between the Fn2 expressed by the formula (2) and the core hardness (HV) after nitriding in the Investigation 6 in the EXAMPLES.

FIG. 16 is a graph summarizing the relationship between the Fn2 expressed by the formula (2) and the indentation deformation amount in the Investigation 9 in the EXAMPLES.

FIG. 17 is a graph summarizing the relationship between the Fn3 expressed by the formula (3) and the surface hardness (HV) after nitriding in the Investigation 6 in the EXAMPLES.

FIG. 18 is a graph summarizing the relationship between the Fn3 expressed by the formula (3) and the rotating bending fatigue strength in the Investigation 7 in the EXAMPLES.

FIG. 19 is a graph summarizing the relationship between the Fn3 expressed by the formula (3) and the wear depth in the Investigation 8 in the EXAMPLES.

#### MODE FOR CARRYING OUT THE INVENTION

In the following, the requirements of the present invention are described in detail. In the following description, the symbol “%” for the content of each element means “% by mass”.

##### (A) Chemical Composition:

C: 0.10 to 0.15%

C (carbon) is an essential element for ensuring the bending fatigue strength and core hardness of the cold-forged/nitrided component, and 0.10% or more of C must be contained. However, if the content of C is too large, the hardness increases, and thereby the cold forgeability and machinability deteriorate. Therefore, the upper limit of the C content is set; and the content of C is set to 0.10 to 0.15%. The content of C is preferably set to 0.13% or less.

Si: not less than 0.02% and less than 0.10%

Si (silicon) has a deoxidizing action. In order to achieve this effect, 0.02% or more of Si must be contained. However, if the content of Si is too large, the hardness increases, and thereby the cold forgeability deteriorates. Therefore, the upper limit of the Si content is set; and the content of Si is set to not less than 0.02% and less than 0.10%. The content of Si is preferably set to 0.03% or more.

Mn: more than 0.90% and not more than 2.50%

Mn (manganese) has an action for ensuring the bending fatigue strength and core hardness of the cold-forged/nitrided component, and also has a deoxidizing action. In order to achieve these effects, more than 0.90% of Mn must be contained. However, if the content of Mn is too large, the hardness increases, and thereby the cold forgeability and the machinability deteriorate. Therefore, the upper limit of the Mn content is set; and the content of Mn is set to more than 0.90% and not more than 2.50%. The content of Mn is preferably set to 1.50% or more, and 2.00% or less.

Cr: 0.80 to 2.0%

Cr (chromium) combines with N at the time of nitriding to produce nitrides, and therefore Cr has effects of increasing the surface hardness in nitriding and of ensuring the bending fatigue strength and wear resistance of the cold-forged/nitrided component. However, if the content of Cr is less than 0.80%, the above-described effects cannot be achieved. On the other hand, if the content of Cr exceeds 2.0%, the steel becomes hard, and thus the cold forgeability and machinability deteriorate. Therefore, the content of Cr is set to 0.80 to 2.0%. The content of Cr is preferably set to 0.90% or more, and 1.5% or less.

V: 0.05 to 0.50%

V (vanadium) combines with C or/and N at the time of nitriding to form carbides, nitrides, and carbo-nitrides, and therefore V has an effect of increasing the surface hardness. In addition, V has an effect of increasing the core hardness by the age hardening action at a nitriding temperature, that is to say, by forming carbides. In order to achieve these effects, 0.05% or more of V must be contained. However, if

the content of V is large, not only the hardness becomes too high, but also the cold forgeability deteriorates. Therefore, the upper limit of the V content is set; and the content of V is set to 0.05 to 0.50%. The content of V is preferably set to 0.10% or more, and 0.40% or less.

Al: 0.01 to 0.07%

Al (aluminum) has a deoxidizing action. In addition, Al combines with N at the time of nitriding to form AlN, and therefore Al has an effect of increasing the surface hardness. In order to achieve these effects, 0.01% or more of Al must be contained. However, if the content of Al is too large, not only hard and coarse Al<sub>2</sub>O<sub>3</sub> is formed and therefore the cold forgeability deteriorates, but also there arises a problem that the effective case depth in nitriding becomes shallow and the bending fatigue strength and pitting strength deteriorate. Therefore, the upper limit of the Al content is set; and the content of Al is set to 0.01 to 0.07%. The content of Al is preferably set to 0.02% or more, and 0.06% or less.

One of the steels for cold forging/nitriding and the steel

20 materials for cold forging/nitriding of the present invention has a chemical composition consisting of aforementioned elements from C to Al with the balance being Fe and impurities. P, S, N and O among the impurities are P: 0.030% or less, S: 0.050% or less, N: 0.0080% or less, and 25 O: 0.0030% or less. Furthermore, this chemical composition satisfies the conditions for the Fn1 to Fn4 described below. Incidentally, as already described, the term “impurities” so referred to in the phrase “Fe and impurities” indicates those elements which come from the raw materials such as ore and scrap, and/or the production environment when the steel material is produced on an industrial scale.

P: 0.030% or less

P (phosphorous) is contained in the steel as an impurity. When the content of P is too large, P which segregated at the 30 grain boundaries sometimes makes the steel brittle. Therefore, the upper limit of the P content is set; and the content of P is set to 0.030% or less. The more preferable P content is 0.020% or less.

S: 0.050% or less

40 S (sulfur) is contained in the steel as an impurity. If S is contained positively, S combines with Mn to form MnS, and therefore S has an effect of improving the machinability. However, if the content of S exceeds 0.050%, coarse MnS is formed, so that the cold forgeability and bending fatigue 45 strength deteriorate. Therefore, the content of S is set to 0.050% or less. The content of S is preferably set to 0.030% or less. Incidentally, in the case where a machinability improving effect is achieved, the content of S is preferably set to 0.003% or more, and further preferably set to 0.005% or more.

N: 0.0080% or less

N (nitrogen) is contained in the steel as an impurity. Together with C, N combines with an element such as V to 55 form carbo-nitrides. If the carbo-nitrides have precipitated at the time of hot rolling, the hardness becomes high, and the cold forgeability deteriorates. In addition, the effect of increasing the core hardness due to age hardening at a nitriding temperature cannot be achieved sufficiently. Therefore, the N content must be restricted; so that the content of 60 N is set to 0.0080% or less. The preferable N content is 0.0070% or less.

O: 0.0030% or less

O (oxygen) is contained in the steel as an impurity. O forms oxide type inclusions and causes a fatigue failure with 65 the inclusions, which become a starting point of the failure; and thus O degrades the bending fatigue strength. If the content of O exceeds 0.0030%, the bending fatigue strength

deteriorates remarkably. Therefore, the content of O is set to 0.0030% or less. Incidentally, the preferable O content is 0.0020% or less.

Another of the steels for cold forging/nitriding and the steel materials for cold forging/nitriding of the present invention has a chemical composition, which contains one or more elements selected from Mo, Cu, Ni, Ti, Nb, Zr, Pb, Ca, Bi, Te, Se and Sb in lieu of a part of Fe mentioned above and satisfies the conditions for the Fn1 to Fn4.

Hereunder, the effects of containing Mo, Cu, Ni, Ti, Nb, Zr, Pb, Ca, Bi, Te, Se and Sb, which are optional elements, and the reasons for the restriction of content thereof are explained.

Mo: 0.50% or less

Mo (molybdenum) combines with C at a nitriding temperature to form carbides, and therefore Mo has an action for increasing the core hardness due to age hardening, so that Mo can be contained to achieve the above effect. However, if Mo is contained exceeding 0.50%, the hardness increases, and thereby the cold forgeability and machinability deteriorate. Therefore, if Mo is contained, the content of Mo is set to 0.50% or less. Incidentally, when Mo is contained, the content of Mo is preferably 0.40% or less.

On the other hand, in the case where Mo is contained, in order to stably achieve the above-described effect of Mo, it is preferable that the content of Mo be 0.05% or more.

Both of Cu and Ni have an action for increasing the core hardness. Therefore, in order to achieve the above effect, these elements can be contained. In the following, the above-mentioned Cu and Ni will be explained.

Cu: 0.50% or less

Cu (copper) has an action for increasing the core hardness, and therefore, in order to achieve the above effect, Cu can be contained. However, if the content of Cu becomes large, the cold forgeability and machinability deteriorate, and additionally at high temperatures under hot rolling and so on, Cu fuses into a liquid. The liquefied Cu permeates into grain boundaries and makes the grain boundaries brittle, and thus causes surface defects in hot rolling. Therefore, if Cu is contained, the upper limit of the Cu content is set; and the content of Cu is set to 0.50% or less. When Cu is contained, the content of Cu is preferably 0.40% or less.

On the other hand, in the case where Cu is contained, in order to stably achieve the above-described effect of Cu, it is preferable that the content of Cu be 0.10% or more.

Ni: 0.50% or less

Ni (nickel) has an action for increasing the core hardness, and therefore, in order to achieve the above effect, Ni can be contained. However, if the content of Ni becomes large, the cold forgeability and machinability deteriorate. Therefore, if Ni is contained, the upper limit of the Ni content is set; and the content of Ni is set to 0.50% or less. When Ni is contained, the content of Ni is preferably 0.40% or less.

On the other hand, in the case where Ni is contained, in order to stably achieve the above-described effect of Ni, it is preferable that the content of Ni be 0.10% or more.

With regard to the aforementioned Cu and Ni, only one or a combination of two or more elements can be contained. The total amount in the case where these elements are contained compositely can be 1.00% when both of the Cu content and the Ni content take the respective upper limit values: however, the said total amount is preferably 0.80% or less. In addition, in the case where Cu is contained, Ni is preferably contained compositely in order to avoid the occurrence of surface defects in hot rolling described above.

All of Ti, Nb and Zr have an action for improving the bending fatigue strength by making the grains fine. There-

fore, in order to achieve the above effect, these elements can be contained. In the following, the aforementioned Ti, Nb and Zr will be explained.

Ti: 0.20% or less

Ti (titanium) combines with C or/and N to form fine carbides, nitrides, and carbo-nitrides which make the grains fine; and thus Ti has an action for improving the bending fatigue strength. Therefore, in order to achieve the above effect, Ti can be contained. However, in the case where the content of Ti is large, coarse TiN is produced, and thus the bending fatigue strength rather deteriorates. Therefore, if Ti is contained, the upper limit of the Ti content is set; and the content of Ti is set to 0.20% or less. When Ti is contained, the content of Ti is preferably 0.10% or less.

On the other hand, in the case where Ti is contained, in order to stably achieve the above-described effect of Ti, it is preferable that the content of Ti be 0.005% or more.

Nb: 0.10% or less

Nb (niobium) combines with C or/and N to form fine carbides, nitrides, and carbo-nitrides which make the grains fine; and thus Nb has an action for improving the bending fatigue strength. Therefore, in order to achieve the above effect, Nb can be contained. However, in the case where the content of Nb is large, the hardness increases, and thereby the cold forgeability and machinability deteriorate. Therefore, if Nb is contained, the upper limit of the Nb content is set; and the content of Nb is set to 0.10% or less. When Nb is contained, the content of Nb is preferably 0.07% or less.

On the other hand, in the case where Nb is contained, in order to stably achieve the above-described effect of Nb, it is preferable that the content of Nb be 0.020% or more.

Zr: 0.10% or less

Zr (zirconium) also combines with C or/and N to form fine carbides, nitrides, and carbo-nitrides which make the grains fine; and thus Zr has an action for improving the bending fatigue strength. Therefore, in order to achieve the above effect, Zr can be contained. However, in the case where the content of Zr is large, the hardness increases, and thereby the cold forgeability and machinability deteriorate. Therefore, if Zr is contained, the upper limit of the Zr content is set; and the content of Zr is set to 0.10% or less. When Zr is contained, the content of Zr is preferably 0.07% or less.

On the other hand, in the case where Zr is contained, in order to stably achieve the above-described effect of Zr, it is preferable that the content of Zr be 0.002% or more.

With regard to the aforementioned Ti, Nb and Zr, only one or a combination of two or more elements can be contained. The total amount in the case where these elements are contained compositely can be 0.40% when all of the contents of Ti, Nb and Zr take the respective upper limit values: however, the said total amount is preferably 0.24% or less.

All of Pb, Ca, Bi, Te, Se and Sb have an action for improving the machinability. Therefore, in order to achieve the above effect, these elements can be contained. In the following, the aforementioned Pb, Ca, Bi, Te, Se and Sb will be explained.

Pb: 0.50% or less

Pb (lead) has an action for improving the machinability. Therefore, in order to achieve the above effect, Pb can be contained. However, in the case where the content of Pb is large, the hot workability deteriorates, and in addition, the toughness of the cold-forged/nitrided component also deteriorates. Therefore, if Pb is contained, the upper limit of the Pb content is set; and the content of Pb is set to 0.50% or less. When Pb is contained, the content of Pb is preferably 0.20% or less.

## 11

On the other hand, in the case where Pb is contained, in order to stably achieve the above-described effect of Pb, it is preferable that the content of Pb be 0.02% or more.

Ca: 0.010% or less

Ca (calcium) has an action for improving the machinability. Therefore, in order to achieve the above effect, Ca can be contained. However, in the case where the content of Ca is large, the hot workability deteriorates, and in addition, the toughness of the cold-forged/nitrided component also deteriorates. Therefore, if Ca is contained, the upper limit of the Ca content is set; and the content of Ca is set to 0.010% or less. When Ca is contained, the content of Ca is preferably 0.005% or less.

On the other hand, in the case where Ca is contained, in order to stably achieve the above-described effect of Ca, it is preferable that the content of Ca be 0.0003% or more.

Bi: 0.30% or less

Bi (bismuth) also has an action for improving the machinability. Therefore, in order to achieve the above effect, Bi can be contained. However, in the case where the content of Bi is large, the hot workability deteriorates, and in addition, the toughness of the cold-forged/nitrided component also deteriorates. Therefore, if Bi is contained, the upper limit of the Bi content is set; and the content of Bi is set to 0.30% or less. When Bi is contained, the content of Bi is preferably 0.10% or less.

On the other hand, in the case where Bi is contained, in order to stably achieve the above-described effect of Bi, it is preferable that the content of Bi be 0.005% or more.

Te: 0.30% or less

Te (tellurium) has an action for improving the machinability. Therefore, in order to achieve the above effect, Te can be contained. However, in the case where the content of Te is large, the hot workability deteriorates, and in addition, the toughness of the cold-forged/nitrided component also deteriorates. Therefore, if Te is contained, the upper limit of the Te content is set; and the content of Te is set to 0.30% or less. When Te is contained, the content of Te is preferably 0.10% or less.

On the other hand, in the case where Te is contained, in order to stably achieve the above-described effect of Te, it is preferable that the content of Te be 0.003% or more.

Se: 0.30% or less

Se (selenium) also has an action for improving the machinability. Therefore, in order to achieve the above effect, Se can be contained. However, in the case where the content of Se is large, the hot workability deteriorates, and in addition, the toughness of the cold-forged/nitrided component also deteriorates. Therefore, if Se is contained, the upper limit of the Se content is set; and the content of Se is set to 0.30% or less. When Se is contained, the content of Se is preferably 0.10% or less.

On the other hand, in the case where Se is contained, in order to stably achieve the above-described effect of Se, it is preferable that the content of Se be 0.005% or more.

Sb: 0.30% or less

Sb (antimony) has an action for improving the machinability. Therefore, in order to achieve the above effect, Sb can be contained. However, in the case where the content of Sb is large, the hot workability deteriorates, and in addition, the toughness of the cold-forged/nitrided component also deteriorates. Therefore, if Sb is contained, the upper limit of the Sb content is set; and the content of Sb is set to 0.30% or less. When Sb is contained, the content of Sb is preferably 0.10% or less.

## 12

On the other hand, in the case where Sb is contained, in order to stably achieve the above-described effect of Sb, it is preferable that the content of Sb be 0.005% or more.

With regard to the aforementioned Pb, Ca, Bi, Te, Se and Sb, only one or a combination of two or more elements can be contained. The total amount in the case where these elements are contained compositely is preferably 0.50% or less, and more preferably 0.30% or less.

Fn1; 35 to 200

With regard to the steel for cold forging/nitriding and the steel material for cold forging/nitriding of the present invention, the Fn1 expressed by the following formula (1) must be 35 to 200;

$$Fn1=Mn/S \quad (1);$$

wherein each symbol Mn and S represents the content by mass percent of the element concerned.

The above Fn1 is a parameter serving as an index of the production of MnS and the center segregation. If the Fn1 is less than 35, the content of S becomes too large, and thereby the production of coarse MnS cannot be prevented. On the other hand, if the Fn1 exceeds 200, the content of Mn becomes too large, and thereby coarse MnS is produced in the center segregation region. In these cases, the bending fatigue strength deteriorates, and in addition, it is difficult to prevent the occurrence of cracks at the time of cold forging. The Fn1 is preferably 40 or more, and 190 or less.

Fn2; 20 to 80

With regard to the steel for cold forging/nitriding and the steel material for cold forging/nitriding of the present invention, the Fn2 expressed by the following formula (2) must be 20 to 80;

$$Fn2=(669.3 \times \log_e C - 1959.6 \times \log_e N - 6983.3) \times (0.067 \times Mo + 0.147 \times V) \quad (2);$$

wherein each symbol C, N, Mo and V represents the content by mass percent of the element concerned.

The above Fn2 is a parameter serving as an index of the amount of age hardening caused by nitriding after cold forging, that is to say, allowance of improvement in the core hardness caused by nitriding. When the Fn2 is 20 or more, the amount of age hardening after nitriding becomes large, and thereby the core hardness increases. However, if the Fn2 exceeds 80, not only the above-described effect is saturated, but also the cold forgeability deteriorates. The Fn2 is preferably 30 or more.

Fn3; 160 or more

With regard to the steel for cold forging/nitriding and the steel material for cold forging/nitriding of the present invention, the Fn3 expressed by the following formula (3) must be 160 or more;

$$Fn3=140 \times Cr + 125 \times Al + 235 \times V \quad (3);$$

wherein each symbol Cr, Al and V represents the content by mass percent of the element concerned.

The above Fn3 is a parameter serving as an index of the surface hardness, bending fatigue strength, and wear resistance after nitriding.

All of Cr, Al and V produce hard nitrides and carbonitrides near the surface of the cold-forged/nitrided component during nitriding treatment, and thereby they can increase the surface hardness. By making the Fn3 160 or more, the surface hardness becomes 700 or more in HV, and the bending fatigue strength and wear resistance equivalent to those of a material performed the treatment of the "carburizing and quenching" are attained. In the case where the Fn3 is less than 160, the surface hardness is low, and the

## 13

bending fatigue strength and wear resistance are poor as compared with the said material performed the treatment of the "carburizing and quenching". The Fn3 is preferably 170 or more, and 350 or less.

Fn4: 150 to 200

With regard to the steel for cold forging/nitriding and the steel material for cold forging/nitriding of the present invention, the Fn4 expressed by the following formula (4) must be 150 to 200;

$$Fn4 = \frac{511 \times C + 33 \times Mn + 56 \times Cu + 15 \times Ni + 36 \times Cr + 5 \times Mo + 134 \times V}{V} \quad (4)$$

wherein each symbol C, Mn, Cu, Ni, Cr, Mo and V represents the content by mass percent of the element concerned.

The Fn4 is a parameter serving as an index of the machinability after cold working

If the Fn4 is 150 to 200, in turning after cold forging, the chip disposability is excellent, and excellent machinability is provided. In the case where the Fn4 is less than 150, the chip produced by turning becomes long, and the chip disposability is poor. In addition, in the case where the Fn4 is more than 200, the cutting resistance in turning becomes high, which causes a deterioration in the tool life. The Fn4 is preferably 160 or more, and 190 or less.

(B) Content of V in Precipitates Determined by the Extraction Residue Analysis:

The steel material for cold forging/nitriding of the present invention is regulated so that in addition to having the chemical composition described in the above item (A), the content of V in precipitates determined by the extraction residue analysis is 0.10% or less.

If fine V precipitates, that is to say, the carbides, nitrides and carbo-nitrides of V do precipitate in the steel material for cold forging/nitriding in a large amount, the ferrite is strengthened and the hardness is increased, so that the cold forgeability is liable to deteriorate. Therefore, in order to ensure the cold forgeability, the content of V in precipitates determined by the extraction residue analysis is set to 0.10% or less. The content of V in precipitates described above is preferably 0.08% or less.

The content of V in precipitates determined by the extraction residue analysis can be determined as described below. For example, first, a proper test piece is cut off. Second, the cut-off test piece is subjected to a constant-current electrolysis in a 10% AA type solution. Third, the extracted solution is filtrated through a filter having a mesh size of 0.2  $\mu$ m. Finally, the filtrated substance is subjected to a general chemical analysis. The 10% AA type solution is a solution in which tetramethylammoniumchloride, acetylacetone, and methanol are mixed in the ratio of 1:10:100.

As described above, in the case where the steel material is as-hot-rolled condition or as-hot-forged condition, the carbides, nitrides, and carbo-nitrides of V had precipitated, and thus in some cases, the cold forgeability is insufficient. Therefore, in order to obtain the steel material for cold forging/nitriding in which the content of V in precipitates determined by the extraction residue analysis is 0.10% or less, it is preferable that the steel material be "normalized"; in the concrete, the steel material be heated to a temperature of, for example, 850 to 950°C. after hot rolling or/and hot forging, and thereafter be cooled to room temperature by a forced air cooling.

After being carried out the heating treatment in the temperature range mentioned above, if the steel material is "normalized" by being cooled to room temperature with an atmospheric cooling or a slow cooling, the carbides, nitrides, and carbo-nitrides of V do precipitate again in the cooling

## 14

process, so that the hardness increases and, in some cases, the cold forgeability deteriorates. Therefore, in order to prevent the carbides, nitrides, and carbo-nitrides of V from precipitating, after being heated, the steel material is preferably cooled by a forced air cooling such that the average cooling rate in the temperature range of, for example, 800 to 500°C. is 0.5 to 5.0°C./second.

(C) Cold-Forged/Nitrided Component:

The cold-forged/nitrided component of the present invention must be such that, in addition to having the chemical composition described in the above item (A), the core hardness thereof is 200 or more in HV, the surface hardness thereof is 700 or more in HV, and the effective case depth thereof is 0.20 mm or more.

In the case where the above conditions are met, the cold-forged/nitrided component is excellent in deformation resistance, bending fatigue strength, and wear resistance; and thus it can be used suitably as a component for machine structural use that is used for an automobile transmission and the like, such as a gear and a pulley for a CVT.

The core hardness is preferably 210 or more, and 400 or less in HV. The surface hardness is preferably 710 or more, and 900 or less in HV. The effective case depth is preferably 0.25 mm or more, and 0.50 mm or less.

(D) Method for Producing the Cold-Forged/Nitrided Component:

For example, in the case where the starting material has a cylindrical shape, the cold-forged/nitrided component described in the above item (C) can be manufactured by subjecting the steel material for cold forging/nitriding having the chemical composition described in the above item (A) and the content of V in precipitates determined by the extraction residue analysis described in the above item (B) to cold forging at a compression ratio of 30% or more, and thereafter by subjecting the steel material to nitriding at a temperature of 400 to 650°C. for 1 to 30 hours. The said compression ratio is a value expressed by the formula of " $\{(H_o - H)/H_o\} \times 100$ ", when the height of starting material before cold forging is taken as  $H_o$ , and the height of the component after cold forging is taken as  $H$ .

In order to increase the core hardness of the said cold-forged/nitrided component, it is preferable to increase the working ratio, that is to say, the strain in cold forging, and to make the most of the strengthening due to work hardening.

After the said cold forging has been carried out, in order to make the most of the strengthening due to age hardening in addition to the said strengthening due to work hardening, it is preferable to carry out nitriding at a temperature of 400 to 650°C. for 1 to 30 hours.

In the case where the nitriding temperature is low and is less than 400°C., although a high surface hardness can be given to the cold-forged/nitrided component, the effective case depth is shallow, and in addition, it is difficult to achieve the increase in core hardness due to age hardening. On the other hand, in the case where the nitriding temperature is high and exceeds 650°C., although the effective case depth of the cold-forged/nitrided component is deep, the surface hardness decreases, and in addition, the core hardness also decreases. The nitriding temperature is preferably 450°C. or more, and 630°C. or less.

Although the nitriding time is changed depending on the effective case depth which is required for the cold-forged/nitrided component, in the case where the nitriding time is less than 1 hour, the effective case depth becomes shallow. On the other hand, in the case where the nitriding time is long and exceeds 30 hours, the cold-forged/nitrided com-

## 15

ponent is unsuitable for mass production. The nitriding time is preferably 1 hour or more, and 20 hours or less.

The method of nitriding for obtaining the cold-forged/nitrided component of the present invention is not regulated especially, and gas nitriding, salt bath nitriding, ion nitriding and the like can be used. In nitrocarburizing, for example, an RX gas is used together with NH<sub>3</sub>, and the treatment can be carried out in an atmosphere in which NH<sub>3</sub> and the RX gas are in the ratio of 1:1.

Although the nitriding time differs depending on the treatment temperature, for example, when nitrocarburizing is carried out at 590° C., nitriding time of 9 hours can provide the surface hardness, core hardness, and effective case depth described in the above item (C).

In addition, when it is desired to restrain the occurrence of brittle compounds, it is preferable to use fluorine gas as the pretreatment of nitriding due to NH<sub>3</sub>, or to use mixed gas of NH<sub>3</sub> and H<sub>2</sub> as the gas for nitriding.

The following examples, which were carried out by gas nitrocarburizing, illustrate the present invention more spe-

## 16

5 specifically. These examples are, however, by no means limited the scope of the present invention.

## EXAMPLES

The steels 1 to 22 having the chemical compositions shown in Table 1 were melted by using a 180 kg vacuum melting furnace and cast to ingots.

The steels 1 to 13 shown in Table 1 are steels of inventive examples with chemical compositions being within the range regulated by the present invention. On the other hand, 15 the steels 14 to 22 are steels of comparative examples with chemical compositions being out of the range regulated by the present invention. Note that, with respect to Mo and V in the Fn2 expressed by the formula (2), V in the Fn3 20 expressed by the formula (3) and Cu, Ni, Mo and V in the Fn4 expressed by the formula (4), each symbol “-” in Table 1 indicates “0 (zero)”.

25 Among the steels of comparative examples mentioned above, the steel 14 is a steel corresponding to the SCr420H specified in JIS G 4052 (2008).

TABLE 1

| Division             | Steel | Chemical composition (% by mass) Balance: Fe and impurities |       |       |       |       |      |      |      |      |
|----------------------|-------|-------------------------------------------------------------|-------|-------|-------|-------|------|------|------|------|
|                      |       | C                                                           | Si    | Mn    | P     | S     | Cu   | Ni   | Cr   | Mo   |
| Inventive examples   | 1     | 0.10                                                        | 0.07  | 1.55  | 0.015 | 0.010 | —    | —    | 0.95 | —    |
|                      | 2     | 0.11                                                        | 0.07  | 1.62  | 0.020 | 0.025 | —    | —    | 1.20 | —    |
|                      | 3     | 0.13                                                        | 0.08  | 1.78  | 0.008 | 0.018 | —    | —    | 0.91 | —    |
|                      | 4     | 0.10                                                        | 0.09  | 1.52  | 0.008 | 0.015 | —    | —    | 0.90 | 0.35 |
|                      | 5     | 0.10                                                        | 0.09  | 1.50  | 0.010 | 0.010 | —    | —    | 1.02 | 0.25 |
|                      | 6     | 0.10                                                        | 0.03  | 1.50  | 0.012 | 0.009 | —    | —    | 0.90 | —    |
|                      | 7     | 0.15                                                        | 0.05  | 1.55  | 0.011 | 0.012 | —    | —    | 1.22 | —    |
|                      | 8     | 0.12                                                        | 0.05  | 1.78  | 0.014 | 0.033 | —    | —    | 0.97 | —    |
|                      | 9     | 0.13                                                        | 0.04  | 1.72  | 0.007 | 0.029 | —    | —    | 1.15 | —    |
|                      | 10    | 0.11                                                        | 0.05  | 2.05  | 0.008 | 0.015 | 0.15 | —    | 0.93 | 0.03 |
|                      | 11    | 0.15                                                        | 0.08  | 1.55  | 0.009 | 0.019 | —    | 0.18 | 1.33 | —    |
|                      | 12    | 0.10                                                        | 0.06  | 1.53  | 0.010 | 0.043 | 0.23 | 0.15 | 1.65 | —    |
|                      | 13    | 0.13                                                        | 0.07  | 1.62  | 0.023 | 0.035 | —    | —    | 1.03 | —    |
| Comparative examples | 14    | *0.18                                                       | *0.16 | *0.75 | 0.017 | 0.020 | —    | —    | 0.95 | —    |
|                      | 15    | *0.16                                                       | 0.08  | 1.87  | 0.016 | 0.010 | —    | —    | 1.39 | —    |
|                      | 16    | 0.13                                                        | 0.05  | 1.50  | 0.017 | 0.050 | —    | —    | 1.25 | —    |
|                      | 17    | 0.12                                                        | 0.07  | 1.97  | 0.027 | 0.007 | —    | —    | 1.32 | 0.42 |
|                      | 18    | 0.10                                                        | 0.09  | 1.51  | 0.011 | 0.013 | —    | —    | 0.88 | —    |
|                      | 19    | 0.14                                                        | 0.08  | 1.65  | 0.012 | 0.015 | —    | —    | 0.93 | 0.45 |
|                      | 20    | 0.12                                                        | 0.07  | 1.52  | 0.012 | 0.012 | —    | —    | 0.92 | —    |
|                      | 21    | 0.10                                                        | 0.03  | 1.50  | 0.009 | 0.008 | —    | —    | 0.96 | —    |
|                      | 22    | 0.10                                                        | 0.08  | 1.51  | 0.012 | 0.010 | —    | —    | 0.80 | —    |

| Division           | Steel | Chemical composition (% by mass) Balance: Fe and impurities |      |        |        |                       |     |     |     |     |
|--------------------|-------|-------------------------------------------------------------|------|--------|--------|-----------------------|-----|-----|-----|-----|
|                    |       | Al                                                          | V    | N      | O      | Others                | Fn1 | Fn2 | Fn3 | Fn4 |
| Inventive examples | 1     | 0.049                                                       | 0.10 | 0.0055 | 0.0010 | —                     | 155 | 25  | 163 | 150 |
|                    | 2     | 0.033                                                       | 0.12 | 0.0060 | 0.0015 | —                     | 65  | 28  | 200 | 169 |
|                    | 3     | 0.035                                                       | 0.13 | 0.0075 | 0.0020 | —                     | 99  | 24  | 162 | 175 |
|                    | 4     | 0.032                                                       | 0.25 | 0.0077 | 0.0010 | —                     | 101 | 61  | 189 | 169 |
|                    | 5     | 0.022                                                       | 0.31 | 0.0075 | 0.0017 | —                     | 150 | 66  | 218 | 180 |
|                    | 6     | 0.028                                                       | 0.38 | 0.0070 | 0.0012 | —                     | 167 | 67  | 219 | 184 |
|                    | 7     | 0.034                                                       | 0.15 | 0.0062 | 0.0015 | —                     | 129 | 38  | 210 | 192 |
|                    | 8     | 0.022                                                       | 0.19 | 0.0059 | 0.0009 | Pb: 0.07, Ca: 0.0015  | 54  | 46  | 183 | 180 |
|                    | 9     | 0.036                                                       | 0.15 | 0.0059 | 0.0010 | Se: 0.05, Sb: 0.06    | 59  | 38  | 201 | 185 |
|                    | 10    | 0.050                                                       | 0.11 | 0.0068 | 0.0021 | Ti: 0.07              | 137 | 24  | 162 | 181 |
|                    | 11    | 0.027                                                       | 0.12 | 0.0052 | 0.0018 | —                     | 82  | 36  | 218 | 194 |
|                    | 12    | 0.029                                                       | 0.09 | 0.0058 | 0.0015 | Zr: 0.039, Te: 0.0025 | 36  | 21  | 256 | 188 |
|                    | 13    | 0.038                                                       | 0.23 | 0.0061 | 0.0012 | Nb: 0.029, Bi: 0.033  | 46  | 56  | 203 | 188 |

TABLE 1-continued

|                      |    |       |       |         |        |   |      |     |      |      |
|----------------------|----|-------|-------|---------|--------|---|------|-----|------|------|
| Comparative examples | 14 | 0.019 | * —   | *0.0130 | 0.0015 | — | 38   | *0  | *135 | 151  |
|                      | 15 | 0.025 | 0.18  | 0.0076  | 0.0013 | — | 187  | 36  | 240  | *218 |
|                      | 16 | 0.030 | 0.20  | 0.0055  | 0.0018 | — | *30  | 54  | 226  | 188  |
|                      | 17 | 0.068 | 0.18  | 0.0067  | 0.0028 | — | *281 | 77  | 236  | 200  |
|                      | 18 | 0.050 | 0.13  | 0.0078  | 0.0024 | — | 116  | *19 | 160  | 150  |
|                      | 19 | 0.036 | 0.12  | 0.0054  | 0.0019 | — | 110  | *92 | 163  | 178  |
|                      | 20 | 0.027 | 0.10  | 0.0050  | 0.0017 | — | 127  | 29  | *156 | 158  |
|                      | 21 | 0.070 | 0.07  | 0.0040  | 0.0019 | — | 188  | 24  | 160  | *145 |
|                      | 22 | 0.023 | *0.52 | 0.0079  | 0.0018 | — | 151  | 74  | 237  | 199  |

Fn1 = Mn/S

Fn2 = (669.3 x log<sub>10</sub>C - 1959.6 x log<sub>10</sub>N - 6983.3) x (0.067 x Mo + 0.147 x V)

Fn3 = 140 x Cr + 125 x Al + 235 x V

Fn4 = 511 x C + 33 x Mn + 56 x Cu + 15 x Ni + 36 x Cr + 5 x Mo + 134 x V

The mark “\*” indicates falling outside the conditions regulated by the present invention.

15

Each ingot was subjected to the homogenizing treatment by being held at 1250°C. for 5 hours, and thereafter was hot forged to prepare both a steel bar having a diameter of 35 mm and a length of 1000 mm and a steel bar having a diameter of 45 mm and a length of 1000 mm.

Among the steel bars mentioned above, the steel bars of the steels 1 to 13 and 15 to 22 were “normalized” by being held at 920°C. for 1 hour and thereafter by being cooled to room temperature by a forced air cooling. As a result of measurement made by inserting a thermocouple in the steel bar, it was revealed that the average cooling rate in the temperature range of 800 to 500°C. of each forced air cooling was 1.40°C./second in the R/2 portion (“R” represents a radius of the steel bar) of the steel bar having the diameter of 35 mm, and 0.74°C./second in the R/2 portion of the steel bar having the diameter of 45 mm.

On the other hand, the steel bars of the steel 14 containing no V were “normalized” by being held at 920°C. for 1 hour and thereafter by being cooled to room temperature by an atmospheric cooling.

With regard to each of the steels, various types of test pieces were cut off from a part of the thus normalized steel bar having the diameter of 35 mm.

In the concrete, with regard to each of the steels, the said normalized steel bar having the diameter of 35 mm was “cut transversely”, that is to say, was cut perpendicularly to the axial direction (the longitudinal direction). Next, the cut steel bar was embedded in a resin so that the cut plane did be the test plane. Thereafter the above embedded steel bar was polished so that the cut plane was mirror-like finished, in order to prepare a test piece for measurement of Vickers hardness as-normalized condition (that is to say, before cold working) and for observation of microstructure.

In addition, with regard to each of the steels, a specimen measuring 10 mm x 10 mm x 10 mm was cut off from the R/2 portion of the said normalized steel bar having the diameter of 35 mm, in order to carry out the extraction residue analysis.

Furthermore, with regard to each of the steels, as test pieces for measuring critical compression ratio at the time of cold forging, 5 notched test pieces shown in FIG. 1 were cut off from the central portion of the said normalized steel bar having the diameter of 35 mm in parallel to the axial direction thereof.

In addition, with regard to each of the steels, a strain was given by cold drawing in place of cold forging, and the properties after cold forging were evaluated by the properties after the drawing.

That is to say, the remainder of the normalized steel bar having the diameter of 35 mm was peeled to a diameter of 30 mm, being subjected to a pickling and lubricating treatment.

ment, and thereafter the said steel bar was carried out the cold drawing so that the diameter became 24 mm.

The diameters of dies used for the above drawing were 28.7 mm, 26.5 mm, and 24 mm in that order. Incidentally, the total reduction of area at the time when drawing was carried out from 30 mm to 24 mm in diameter was 36%.

With regard to each of the steels, the thus obtained cold drawn material having the diameter of 24 mm was cut transversely. Next, the cut material was embedded in a resin so that the cut plane did be the test plane. Thereafter the above embedded material was polished so that the cut plane was mirror-like finished, in order to prepare a test piece for measurement of Vickers hardness after drawing (that is to say, after cold working)

Furthermore, with regard to each of the steels, a round bar test piece having a diameter of 10 mm shown in FIG. 2 for measuring the hardness and so on after nitriding and a notched Ono type rotating bending fatigue test piece having the rough shape shown in FIG. 3 were cut off from the central portion of the said cold drawn material having the diameter of 24 mm in parallel to the axial direction thereof.

Similarly, from the central portion of the said cold drawn material, in parallel to the axial direction thereof, a block test specimen measuring 15.75 mm long, 10.16 mm wide, and 6.35 mm thick (hereinafter, referred to the “block test specimen A”) shown in FIG. 4 and a block test specimen measuring 25 mm long, 5 mm wide, and 12.5 mm thick (hereinafter, referred to the “block test specimen B”) shown in FIG. 5 were cut off.

Except for the symbols “3.2S”, the units of the dimensions that units are not indicated in the above cut-off test pieces shown in FIGS. 1 to 5 are “mm”. The inverted triangular finish marks of three kinds shown in the figures are the “triangular symbols” designating surface roughness described in Explanation Table 1 of JIS B 0601 (1982).

The symbols “3.2S” described with the finish marks in FIG. 3 mean that the maximum height  $R_{max}$  is 3.2  $\mu m$  or less. The indications of “ $R_q$ : 0.10 to 0.20  $\mu m$ ” described with the finish marks in FIGS. 4 and 5 mean that the root-mean-square roughness “ $R_q$ ” specified in JIS B 0601 (2001) is 0.10 to 0.20  $\mu m$ .

On the other hand, the normalized steel bar having the diameter of 45 mm was peeled to a diameter of 35 mm, being subjected to a pickling and lubricating treatment, and thereafter the said steel bar was carried out the cold drawing so that the diameter became 28 mm.

The diameters of dies used for the above drawing were 32.88 mm, 31 mm, and 28 mm in that order. Incidentally, the total reduction of area at the time when drawing was carried out from 35 mm to 28 mm in diameter was 36%.

With regard to each of the steels, the thus obtained cold drawn material having the diameter of 28 mm was cut to a length of 300 mm in order to prepare a test piece for investigation of machinability after drawing (that is to say, after cold working).

The diameters of dies used for the above drawing were 32.88 mm, 31 mm, and 28 mm in that order. Incidentally, the total reduction of area at the time when drawing was carried out from 35 mm to 28 mm in diameter was 36%.

With regard to each of the steels, the thus obtained cold drawn material having the diameter of 28 mm was cut to a length of 300 mm in order to prepare a test piece for investigation of machinability after drawing (that is to say, after cold working).

Among the thus prepared test pieces, the round bar test pieces having a diameter of 10 mm for measuring hardness and so on after nitriding, the notched Ono type rotating bending fatigue test pieces having the rough shape, the block test pieces A, and the block test pieces B were treated by nitriding. In the concrete, the "gas nitrocarburizing" using the heat pattern shown in FIG. 6 was carried out. Incidentally, the "120° C. Oil Cooling" in FIG. 6 means that the test pieces were cooled by being put in the oil having a temperature of 120° C.

The aforementioned notched Ono type rotating bending fatigue test pieces having the rough shape subjected to the said "gas nitrocarburizing" were finished to prepare the notched Ono type rotating bending fatigue test pieces shown in FIG. 7.

The units of the dimensions in the notched Ono type rotating bending fatigue test piece shown in FIG. 7 are "mm". In addition, similarly in the above FIGS. 1 to 5, the inverted triangular finish marks of two kinds shown in FIG. 7 are the "triangular symbols" designating surface roughness described in Explanatory Table 1 of JIS B 0601 (1982).

The "-(wave dash)", which is "waveform symbol", in FIG. 7 means that the surface is not carried out a removal treatment, that is to say, the surface is "as-gas nitrocarburized condition".

By using the thus prepared test pieces, the tests described below were carried out.

Investigation 1: Vickers Hardness Test Before Cold Working

Being based on the "Vickers hardness test—Test method" described in JIS Z 2244 (2009), at a total of 5 points of 1 point in the central portion of the mirror-like finished each test piece for measurement of Vickers hardness before cold working and 4 points in the R/2 portion thereof, Vickers hardness was measured by using a Vickers hardness tester with the testing force being 9.8N; and the arithmetic mean value of the said 5 points was defined as the hardness before cold working.

Investigation 2: Extraction Residue Analysis

The specimens measuring 10 mm×10 mm×10 mm, which were cut off in order to carry out the extraction residue analysis, were electrolyzed at a constant current in a 10% AA type solution. That is to say, in order to remove the accretions on the surface, first, pre-electrolysis was carried out on the specimen under the conditions of electric current: 1000 mA and time: 28 minutes. Thereafter, the accretions on the surface of the specimen were ultrasonically cleaned in alcohol and were removed from the specimen; and further, the mass of the specimen from which accretions had been removed was measured. The thus measured mass was defined as the mass of the specimen before the electrolysis being carried out in the next process.

Next, the specimen was electrolyzed under the conditions of electric current: 173 mA and time: 142 minutes. The thus electrolyzed specimen was taken out, and then, the accretions (residues) on the surface of the specimen were ultrasonically cleaned in alcohol and were removed from the specimen. Thereafter, in order to sample the residues, both the solution after the electrolysis and the solution having been used for ultrasonic cleaning were suction-filtrated through a filter having a mesh size of 0.2 µm; and then, the mass of the specimen from which accretions (residues) had been removed was measured, and the thus measured mass was defined as the mass of the specimen after the electrolysis. From the difference between measured values of specimen masses before and after the electrolysis, the "mass of the electrolyzed portion of the specimen" was determined.

The residues sampled on the filter were shifted onto a petri dish and were dried, and after the mass had been measured, the residues were subjected to an acidolysis treatment.

The solution subjected to the above acidolysis was analyzed by using an ICP emission analyzer (high-frequency inductively coupled plasma emission spectrophotometer) to determine the "mass of V in residues".

With regard to each of the steels, a value that was obtained by dividing the thus obtained "mass of V in residues" by the said "mass of the electrolyzed portion of the specimen", and by being represented in percentage was defined as the "content of V in precipitates determined by the extraction residue analysis".

Investigation 3: Vickers Hardness Test after Cold Working

Similarly in the above "Investigation 1", being based on JIS Z 2244 (2009), at a total of 5 points of 1 point in the central portion of the mirror-like finished each test piece for measurement of Vickers hardness after cold working and 4 points in the R/2 portion thereof, Vickers hardness was measured by using a Vickers hardness tester with the testing force being 9.8N; and the arithmetic mean value of the said 5 points was defined as the hardness after cold working.

Investigation 4: Measurement of the Critical Compression Ratio in Cold Forging

The notched test pieces shown in FIG. 1 were cold compressed until a crack occurred in the notched portion under the macroscopic observation, and the compression ratio at the time of crack occurrence was determined. With regard to each of 5 test pieces, the compression ratio at the time of crack occurrence was determined respectively; and the compression ratio of the third test piece at the time when the 5 test pieces were arranged in ascending order of compression ratio was defined as the critical compression ratio. In the case where the thus defined critical compression ratio was 60% or more, the cold forgeability was supposed to be excellent, and so this value was defined as the target.

Investigation 5: Machinability Test

Using an NC lathe, the machinability was investigated by turning the outer circumference portion of a test piece that had been cold drawn so as to have a diameter of 28 mm and thereafter had been cut to a length of 300 mm.

The above turning was carried out by using a cemented carbide tool consisting mainly of WC, not provided with a chip breaker, under the conditions of cutting speed: 150 m/min, depth of cut: 0.2 mm, and feed rate: 0.8 mm/rev, and in the state of being lubricated with a water-soluble lubricant. The machinability after cold working was evaluated by the chip disposability at the time of turning.

The chip disposability was evaluated as described below. With regard to each of the steels, from optional 10 chips after turning, a chip in which the chip length shown in FIG.

8 was at a maximum was selected, and in order to evaluate the chip disposability, the length thereof was measured. The chip disposability was evaluated as "Excellent (○○)", "Good (○)", and "Poor (x)" in the case where the chip length was not more than 5 mm, in the case where it was more than 5 mm and not more than 10 mm, and in the case where it was more than 10 mm, respectively.

In the case where the chip disposability was evaluated as Excellent or Good (○○ or ○), the machinability was supposed to be excellent, and so this evaluation was defined as the target.

Investigation 6: Measurement of the Core Hardness, Surface Hardness, and Effective Case Depth after Nitriding

The round bar test piece having a diameter of 10 mm which had been subjected to the said gas nitrocarburizing was cut transversely. Next, the cut round bar test piece was embedded in a resin so that the cut plane did be the test plane. Thereafter the cut round bar test piece was polished so that the cut plane was mirror-like finished, and the core hardness was measured using a Vickers hardness tester. In addition, by using a micro-Vickers tester, the surface hardness and the effective case depth were investigated.

In the concrete, being based on JIS Z 2244 (2009), at a total of 5 points of 1 point in the central portion of the mirror-like finished test piece and 4 points in the R/2 portion thereof, Vickers hardness was measured by using the Vickers hardness tester with the testing force being 9.8N, and the arithmetic mean value of the said 5 points was defined as the "core hardness".

Similarly in the above-described case, being based on JIS Z 2244 (2009), by using the same embedded test piece, at optional 10 points at a position 0.01 mm deep from the surface of each test piece, HV was measured by using the micro-Vickers tester with the testing force being 0.98N, and the arithmetic mean value of the ten points was defined as the "surface hardness".

Furthermore, by using the same embedded test piece, being based on JIS Z 2244 (2009), HV were measured successively from the surface of the mirror-like finished test piece by using the micro-Vickers tester with the testing force being 1.96N, and the hardness distribution map was prepared. The distance from the surface to the position at which HV did be 550 was defined as the "effective case depth".

Investigation 7: Ono Type Rotating Bending Fatigue Test

By using Ono type rotating bending fatigue test pieces having been finished after the said gas nitrocarburizing, the Ono type rotating bending fatigue test was carried out under the test conditions described below, and the maximum strength at which the test piece did not rupture in the number of cycles of  $10^7$  was defined as the "rotating bending fatigue strength". In the case where the rotating bending fatigue strength was 500 MPa or more, the thus defined rotating bending fatigue strength was supposed to be excellent, and so this value was defined as the target.

Temperature: room temperature,

Atmosphere: in the air,

Number of revolutions: 3000 rpm.

Investigation 8: Investigation of the Wear Resistance

The wear resistance was investigated by the block-on-ring wear test. That is to say, as shown in FIG. 9, the plane having a length of 15.75 mm and a thickness of 6.35 mm (hereinafter, referred to as the "test plane") of the said gas nitrocarburized block test piece A was pushed against a ring test piece, and the said ring test piece was rotated, whereby the wear test was carried out.

In the concrete, 100 milliliters of a commercial automatic transmission oil was put in a test chamber as a lubricating

oil, the temperature thereof being raised to 90° C., thereafter the test plane of the block test piece A was pushed against the ring test piece with a testing force of 1000N, and the ring test piece was rotated until the total slipping distance became 8000 m with the slipping velocity being 0.1 m/sec-ond.

The above ring test piece was prepared as described below. From a steel bar having a diameter of 45 mm of SCM420 specified in JIS G 4053 (2008), a test piece approximately having the shape shown in FIG. 10 was cut off with the axial direction thereof being aligned with the steel bar, and the said cut-off test piece was subjected to the gas "carburizing and quenching" and tempering with the heat patterns shown in FIG. 11, thereafter the outer circumference portion thereof being ground by 100  $\mu\text{m}$ , and thereby the test piece was finished to the size and shape shown in FIG. 10.

The units of the dimensions that units are not indicated in the above ring test piece shown in FIG. 10 are "mm", and the inverted triangular finish mark shown in the said FIG. 10 is the "triangular symbol" designating surface roughness described in Explanation Table 1 of JIS B 0601 (1982). In addition, the "Rq: 0.15 to 0.35  $\mu\text{m}$ " attached to the said finish mark means that the root-mean-square roughness "Rq" specified in JIS B 0601 (2001) is 0.15 to 0.35  $\mu\text{m}$ .

The "Cp" in FIG. 11 represents carbon potential. In addition, the "80° C. Oil Cooling" means that the ring test piece was cooled by being put in the oil having a temperature of 80° C.

After the finish of the said block-on-ring wear test, by using a surface roughness tester, the surface roughness of the test plane of the block test piece A was measured continuously in the order of non-contact portion, contact portion, and non-contact portion as indicated by arrow marks 1, 2, and 3 in FIG. 12. And then, in the obtained each cross-sectional curve, the largest difference between the non-contact portion and the contact portion was defined as an each wear depth. With regard to the each block test piece A, three wear depths were determined, and the mean value thereof was defined as the wear depth. In the case where the thus defined wear depth was 10.0  $\mu\text{m}$  or less, the wear resistance was supposed to be excellent, and so this value was defined as the target.

The "non-contact portion" and "contact portion" mentioned above means the "non-contact portion" and "contact portion" with the ring test piece.

Investigation 9: Investigation of the Deformation Resistance

The deformation resistance was investigated by an indentation test. That is to say, as shown in FIG. 13, an indentation test jig having the shape shown in FIG. 14 was pushed into the plane having a length of 25 mm and a thickness of 12.5 mm (hereinafter, referred to as the "test plane") of the said gas nitrocarburized block test piece B, whereby the deformation resistance was investigated. The said indentation test jig was prepared as described below like the ring test piece for the block-on-ring wear test. From a steel bar having a diameter of 45 mm of SCM420 specified in JIS G 4053 (2008), a test piece approximately having the shape shown in FIG. 14 was cut off with the axial direction thereof being aligned with the steel bar. The said cut-off test piece was subjected to the gas "carburizing and quenching" and tempering with the heat patterns shown in FIG. 11, thereafter the outer circumference portion thereof being ground by 100  $\mu\text{m}$ , and thereby the test piece was finished to the size and shape shown in FIG. 14.

In the concrete, by using an oil hydraulic servo testing machine, the indentation test jig was pushed into the test plane of the block test piece B with a testing force of 5000N. After the testing force had been relieved, similarly in the Investigation 8, the indentation deformation amount in the test plane of the block test piece B was measured in three locations by using the surface roughness tester, and the mean value of three locations was defined as the indentation deformation amount. In the case where the thus defined indentation deformation amount was 5.0  $\mu\text{m}$  or less, the deformation resistance was supposed to be excellent, and so this value was defined as the target.

In addition, the relationship between the Fn2 and the core hardness (HV) after nitriding in the Investigation 6 and the relationship between the Fn2 and the indentation deformation amount in the Investigation 9 are summarized in FIGS. 5 15 and 16, respectively.

FIGS. 17 to 19 summarize the relationship between the Fn3 and the surface hardness (HV) after nitriding in the Investigation 6, the relationship between the Fn3 and the rotating bending fatigue strength in the Investigation 7, and the relationship between the Fn3 and the wear depth in the Investigation 8, respectively.

TABLE 2

| Division             | Test No. | Steel | Content of V in precipitates (%) | HV before cold working | HV after cold working | Cold forgeability [critical compression ratio (%)] | Ma-chinability [chip disposability] | Hardness after nitriding |                        | Age hardening                                 |                 | Ef-fective case depth (mm) | Rotat-ing bending fatigue strength (MPa) | Wear depth ( $\mu\text{m}$ ) | Inden-tation deformation amount ( $\mu\text{m}$ ) |
|----------------------|----------|-------|----------------------------------|------------------------|-----------------------|----------------------------------------------------|-------------------------------------|--------------------------|------------------------|-----------------------------------------------|-----------------|----------------------------|------------------------------------------|------------------------------|---------------------------------------------------|
|                      |          |       |                                  |                        |                       |                                                    |                                     | Core hardness [HV]       | Sur-face hardness [HV] | amount due to nitriding [ $\Delta\text{HV}$ ] | case depth (mm) |                            |                                          |                              |                                                   |
|                      |          |       |                                  |                        |                       |                                                    |                                     |                          |                        |                                               |                 |                            |                                          |                              |                                                   |
| Inventive examples   | 1        | 1     | 0.02                             | 198                    | 225                   | 65                                                 | ○                                   | 245                      | 705                    | 20                                            | 0.30            | 540                        | 7.4                                      | 4.0                          |                                                   |
|                      | 2        | 2     | 0.03                             | 232                    | 250                   | 62                                                 | ○                                   | 271                      | 755                    | 21                                            | 0.32            | 590                        | 6.5                                      | 3.6                          |                                                   |
|                      | 3        | 3     | 0.02                             | 230                    | 256                   | 62                                                 | ○                                   | 280                      | 708                    | 24                                            | 0.34            | 570                        | 7.3                                      | 3.0                          |                                                   |
|                      | 4        | 4     | 0.06                             | 240                    | 267                   | 61                                                 | ○                                   | 304                      | 745                    | 37                                            | 0.37            | 520                        | 6.7                                      | 3.0                          |                                                   |
|                      | 5        | 5     | 0.07                             | 240                    | 270                   | 62                                                 | ○                                   | 310                      | 755                    | 40                                            | 0.42            | 610                        | 6.4                                      | 2.9                          |                                                   |
|                      | 6        | 6     | 0.09                             | 198                    | 230                   | 65                                                 | ○                                   | 275                      | 763                    | 45                                            | 0.48            | 620                        | 6.3                                      | 2.9                          |                                                   |
|                      | 7        | 7     | 0.03                             | 239                    | 270                   | 62                                                 | ○                                   | 295                      | 732                    | 25                                            | 0.32            | 540                        | 7.0                                      | 2.8                          |                                                   |
|                      | 8        | 8     | 0.04                             | 230                    | 255                   | 61                                                 | ○○                                  | 281                      | 728                    | 26                                            | 0.36            | 540                        | 7.1                                      | 3.2                          |                                                   |
|                      | 9        | 9     | 0.03                             | 242                    | 262                   | 61                                                 | ○○                                  | 283                      | 741                    | 21                                            | 0.32            | 550                        | 6.8                                      | 3.2                          |                                                   |
|                      | 10       | 10    | 0.02                             | 249                    | 269                   | 62                                                 | ○                                   | 285                      | 720                    | 16                                            | 0.30            | 540                        | 6.6                                      | 3.2                          |                                                   |
|                      | 11       | 11    | 0.04                             | 248                    | 269                   | 62                                                 | ○                                   | 286                      | 742                    | 17                                            | 0.33            | 580                        | 6.8                                      | 3.3                          |                                                   |
|                      | 12       | 12    | 0.03                             | 250                    | 271                   | 61                                                 | ○○                                  | 288                      | 799                    | 17                                            | 0.28            | 610                        | 5.7                                      | 3.1                          |                                                   |
|                      | 13       | 13    | 0.04                             | 232                    | 253                   | 62                                                 | ○○                                  | 272                      | 736                    | 19                                            | 0.38            | 590                        | 6.7                                      | 3.5                          |                                                   |
| Comparative examples | 14       | * 14  | —                                | 176                    | 200                   | # 58                                               | ○                                   | \$195                    | \$552                  | -5                                            | \$0.16          | # 360                      | # 12.6                                   | # 5.6                        |                                                   |
|                      | 15       | * 15  | 0.03                             | 288                    | 305                   | # 55                                               | ○                                   | 325                      | 767                    | 20                                            | 0.32            | 600                        | 6.2                                      | 2.5                          |                                                   |
|                      | 16       | * 16  | 0.04                             | 240                    | 262                   | # 58                                               | ○                                   | 282                      | 757                    | 20                                            | 0.33            | # 480                      | 6.4                                      | 2.8                          |                                                   |
|                      | 17       | * 17  | 0.04                             | 285                    | 305                   | # 55                                               | ○                                   | 334                      | 775                    | 29                                            | 0.32            | # 490                      | 6.1                                      | 2.4                          |                                                   |
|                      | 18       | * 18  | 0.03                             | 182                    | 225                   | 63                                                 | ○                                   | \$197                    | 705                    | -28                                           | 0.30            | 530                        | 7.3                                      | # 5.2                        |                                                   |
|                      | 19       | * 19  | 0.02                             | 278                    | 298                   | # 56                                               | ○                                   | 333                      | 779                    | 35                                            | 0.29            | 610                        | 6.1                                      | 2.3                          |                                                   |
|                      | 20       | * 20  | 0.02                             | 202                    | 220                   | 62                                                 | ○                                   | 240                      | \$678                  | 20                                            | 0.22            | # 440                      | # 10.7                                   | 3.9                          |                                                   |
|                      | 21       | * 21  | 0.01                             | 201                    | 218                   | 62                                                 | # x                                 | 231                      | 712                    | 13                                            | 0.21            | 560                        | 6.6                                      | 4.2                          |                                                   |
|                      | 22       | * 22  | ** 0.13                          | 265                    | 279                   | # 53                                               | ○                                   | 335                      | 782                    | 56                                            | 0.34            | 620                        | 5.8                                      | 2.2                          |                                                   |

With regard to the Test No.14, the steel 14 did contain no V; thus the mark “—” in the column of “Content of V in precipitates” denotes that V was not detected in the precipitates.

“Age hardening amount due to nitriding” indicates the difference between the core hardness (HV) after nitriding and the hardness (HV) after cold working.

The mark “\*” indicates falling outside the conditions of chemical composition regulated by the present invention.

The mark “\*\*” indicates falling outside the condition of “Content of V in precipitates determined by the extraction residue analysis” regulated by the present invention.

The mark “S” indicates falling outside the conditions of the properties after nitriding regulated by the present invention.

The mark “#” indicates falling short of the target in the present invention.

The units of the dimensions that units are not indicated in the above indentation test jig shown in FIG. 14 are “mm”, and the inverted triangular finish mark shown in the said FIG. 14 is the “triangular symbol” designating surface roughness described in Explanation Table 1 of JIS B 0601 (1982). In addition, the “Rq: 0.10 to 0.20  $\mu\text{m}$ ” attached to the said finish mark means that the root-mean-square roughness “Rq” specified in JIS B 0601 (2001) is 0.10 to 0.20  $\mu\text{m}$ .

The test results of the Investigations 1 to 9 are collectively shown in Table 2. In the case where the steel 14 containing no V was used, V was not found in precipitates determined by the extraction residue analysis. Therefore, in the column of the “Content of V in precipitates” of test No. 14, the content of V is described as “-”. In addition, the difference between the core hardness (HV) after nitriding and the hardness (HV) after cold working, which is hardness before nitriding, is given as the age hardening amount ( $\Delta\text{HV}$ ) due to nitriding.

50 From Table 2, it is apparent that, in the case of test Nos. 1 to 13 of the “inventive examples” in which the starting material before nitriding satisfied the conditions regulated by the present invention, both excellent cold forgeability and excellent machinability after cold working were ensured. Moreover, in the case of the said test numbers, all conditions of the core hardness, surface hardness, and effective case depth regulated by the present invention were satisfied after nitriding, and thus excellent deformation resistance, high 55 rotating bending fatigue strength and excellent wear resistance were ensured.

It is apparent that, among the “inventive examples”, in the case of test Nos. 8, 9, 12 and 13, in which the steel 8 containing Pb and Ca, the steel 9 containing Se and Sb, the 60 steel 12 containing Te, and the steel 13 containing Bi were used respectively, the machinability after cold working was especially excellent.

In contrast, in the case of test No. 14 of the "comparative example", the contents of C, Si and N of the used steel 14 were so large as to exceed the range regulated by the present invention; thus the critical compression ratio was as low as 58% and the cold forgeability was poor. In addition, the Fn2 of the steel 14 was zero and deviated from the range of "20 to 80" regulated by the present invention, and the core hardness after nitriding was 195 in HV which was lower than the value regulated by the present invention; thus the deformation resistance was poor, that is to say in the concrete, the indentation deformation amount was as large as 5.6  $\mu\text{m}$ . Furthermore, with regard to the steel 14, the content of Mn was lower than the range regulated by the present invention, V was not contained and the Fn3 was 135, that is to say, the contents of Mn and V and the value of Fn3 deviate from the conditions regulated by the present invention, and in addition, the surface hardness after nitriding was 552 in HV which was lower than the value regulated by the present invention, and the effective case depth after nitriding was 0.16 mm, which was smaller than the value regulated by the present invention; thus the rotating bending fatigue strength was as low as 360 MPa, and moreover the wear resistance was poor, that is to say in the concrete, the wear depth was as large as 12.6  $\mu\text{m}$ .

In the case of test No. 15, the content of C of the used steel 15 was as high as 0.16%, which was higher than the range regulated by the present invention; thus the critical compression ratio was as low as 55% and the cold forgeability was poor. In addition, the Fn4 was as high as 218, which was higher than the range regulated by the present invention. Thus, the cutting resistance in turning becomes high, which may cause a deterioration in the tool life.

In the case of test No. 16, the Fn1 of the used steel 16 was 30 and deviated from the range regulated by the present invention; thus the rotating bending fatigue strength was as low as 480 MPa, and moreover the cold forgeability was poor, that is to say in the concrete, the critical compression ratio was as low as 58%.

In the case of test No. 17, the Fn1 of the used steel 17 was 281 and deviated from the range regulated by the present invention; thus the rotating bending fatigue strength was as low as 490 MPa, and moreover the cold forgeability was poor, that is to say in the concrete, the critical compression ratio was as low as 58%.

In the case of test No. 18, the Fn2 of the used steel 18 was 19 and deviated from the range regulated by the present invention, the core hardness after nitriding was 197 in HV, which was lower than the value regulated by the present invention. Consequently, the deformation resistance was poor, that is to say in the concrete, the indentation deformation amount was as large as 5.2  $\mu\text{m}$ .

In the case of test No. 19, the Fn2 of the used steel 19 was 92 and deviated from the range regulated by the present invention; thus the critical compression ratio was as low as 56% and the cold forgeability was poor.

In the case of test No. 20, the Fn3 of the used steel 20 was as low as 156 and deviated from the restriction of the present invention, and in addition, the surface hardness after nitriding was 678 in HV, which was lower than the value regulated by the present invention; and thus the rotating bending fatigue strength was as low as 440 MPa, and moreover the wear resistance was poor, that is to say in the concrete, the wear depth was as large as 10.7  $\mu\text{m}$ .

In the case of test No. 21, the Fn4 of the used steel 21 was as low as 145 and deviated from the restriction of the present invention, thus the chip disposability was poor.

In the case of test No. 22, the content of V of the used steel 22 was as high as 0.52% and deviated from the restriction of the present invention, and in addition, the content of V in precipitates determined by the extraction residue analysis was as high as 0.13% and deviated from the restriction of the present invention; thus the critical compression ratio was as low as 53% and the cold forgeability was poor.

#### INDUSTRIAL APPLICABILITY

The steel for cold forging/nitriding and the steel material for cold forging/nitriding of the present invention are excellent in cold forgeability and machinability (particularly, chip disposability) after cold forging, and also can provide a component subjected to a cold forging and nitriding treatment with high core hardness and high surface hardness and a large effective case depth. Therefore, the steel for cold forging/nitriding and the steel material for cold forging/nitriding of the present invention are used suitably as a starting material for a cold-forged/nitrided component.

In addition, the cold-forged/nitrided component of the present invention is excellent in deformation resistance, bending fatigue strength, and wear resistance; and therefore it can be used suitably as a component for machine structural use that is used for an automobile transmission and the like, such as a gear and a pulley for a CVT.

The invention claimed is:

1. A steel for cold forging and nitriding, having a chemical composition comprising, by mass percent, C: 0.10 to 0.15%, Si: not less than 0.02% and less than 0.10%, Mn: more than 0.90% and not more than 2.50%, Cr: 0.80 to 2.0%, V: 0.05 to 0.50%, and Al: 0.01 to 0.07%, with the balance being Fe and impurities, wherein

P, S, N and O among the impurities are P: 0.030% or less, S: 0.050% or less, N: 0.0080% or less, and O: 0.0030% or less,

the Fn1 expressed by the formula (1) described below is 35 to 200,

the Fn2 expressed by the formula (2) described below is 20 to 80,

the Fn3 expressed by the formula (3) described below is 160 or more, and

the Fn4 expressed by the formula (4) described below is 150 to 200:

$$\text{Fn1} = \text{Mn/S} \quad (1);$$

$$\text{Fn2} = (669.3 \times \log_e \text{C} - 1959.6 \times \log_e \text{N} - 6983.3) \times (0.067 \times \text{Mo} + 0.147 \times \text{V}) \quad (2);$$

$$\text{Fn3} = 140 \times \text{Cr} + 125 \times \text{Al} + 235 \times \text{V} \quad (3); \text{ and}$$

$$\text{Fn4} = 511 \times \text{C} + 33 \times \text{Mn} + 56 \times \text{Cu} + 15 \times \text{Ni} + 36 \times \text{Cr} + 5 \times \text{Mo} + 134 \times \text{V} \quad (4);$$

where, each symbol C, Mn, S, Cr, Mo, V, N, Al, Cu and Ni in the above formulas (1) to (4) represents the content by mass percent of the element concerned.

2. A steel for cold forging and nitriding, having a chemical composition comprising, by mass percent, C: 0.10 to 0.15%, Si: not less than 0.02% and less than 0.10%, Mn: more than 0.90% and not more than 2.50%, Cr: 0.80 to 2.0%, V: 0.05 to 0.50%, Al: 0.01 to 0.07%, and one or more elements selected from the groups (a) to (d) listed below, with the balance being Fe and impurities, wherein

P, S, N and O among the impurities are P: 0.030% or less, S: 0.050% or less, N: 0.0080% or less, and O: 0.0030% or less,

## 27

the Fn1 expressed by the formula (1) described below is 35 to 200,

the Fn2 expressed by the formula (2) described below is 20 to 80,

the Fn3 expressed by the formula (3) described below is 5 160 or more, and

the Fn4 expressed by the formula (4) described below is 150 to 200:

$$Fn1=Mn/S$$

(1); 10

$$Fn2=(669.3 \times \log_e C - 1959.6 \times \log_e N - 6983.3) \times (0.067 \times Mo + 0.147 \times V)$$

(2),

$$Fn3=140 \times Cr + 125 \times Al + 235 \times V$$

(3); and 15

$$Fn4=511 \times C + 33 \times Mn + 56 \times Cu + 15 \times Ni + 36 \times Cr + 5 \times Mo + 134 \times V$$

(4);

where, each symbol C, Mn, S, Cr, Mo, V, N, Al, Cu and Ni in the above formulas (1) to (4) represents the content by mass percent of the element concerned; 20

(a) Mo: 0.50% or less;

(b) One or more selected from Cu: 0.50% or less and Ni: 0.50% or less;

## 28

(c) One or more selected from Ti: 0.20% or less, Nb: 0.10% or less, and Zr: 0.10% or less;

(d) One or more selected from Pb: 0.50% or less, Ca: 0.010% or less, Bi: 0.30% or less, Te: 0.30% or less, Se: 0.30% or less, and Sb: 0.30% or less.

3. A steel material for cold forging and nitriding having a chemical composition according to claim 1, wherein the content of V in precipitates determined by an extraction residue analysis is 0.10% or less.

4. A steel material for cold forging and nitriding having a chemical composition according to claim 2, wherein the content of V in precipitates determined by an extraction residue analysis is 0.10% or less.

5. A cold forged and nitrided component having a chemical composition according to claim 1, wherein the core hardness thereof is 200 or more in Vickers hardness, the surface hardness thereof is 700 or more in Vickers hardness, and the effective case depth thereof is 0.20 mm or more.

6. A cold forged and nitrided component having a chemical composition according to claim 2, wherein the core hardness thereof is 200 or more in Vickers hardness, the surface hardness thereof is 700 or more in Vickers hardness, and the effective case depth thereof is 0.20 mm or more.

\* \* \* \* \*